

June 28, 1932.

G. A. RICHTER

1,864,619

CYCLIC PROCESS OF FIBER LIBERATION

Filed Sept. 30, 1925



## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## CYCLIC PROCESS OF FIBER LIBERATION

Application filed September 30, 1925. Serial No. 59,583.

This invention relates to the production of a cellulose pulp suitable for conversion into a paper which has a strength approximating that made from "sulphate" or kraft pulps 5 so-called, and has for its salient object to provide a cyclic process for such pulp production through the use of a cooking liquor comprising essentially a mixture of sodium sulphite, sodium sulphide and caustic soda. 10 In certain cases, if desired, either of the alkaline constituents, i. e., the caustic soda or the sodium sulphide, may be omitted from the cooking liquor and the percentages of the other constituents so adjusted as to yield a 15 pulp substantially equivalent to that resulting from a liquor containing all the constituents. In any event, however, the raw cellulosic material, e. g., wood chips, is digested in an alkaline solution of sodium sulphite, 20 the alkalinity being afforded by the sodium hydroxide, the sodium sulphide, or both these alkaline constituents.

In attaining the hereinbefore designated object, this invention provides for the recovery of the mineral or inorganic content 25 of the spent cooking liquor in the form of chemicals which may be reutilized in the preparation of fresh cooking liquor. A feature incident to the use of a digesting liquor such as herein employed is that I am able 30 to dispense with the use of lime, which, however, must be employed in the sulphate process in the causticization of the soda ash recovered by the smelting of the concentrated 35 spent digesting liquor.

In the practice of the present invention, the various constituents of the cooking liquor are used in suitable proportion to effect a 40 liberation of fiber, and the cooking or digesting operation is carried out at the desired temperature and under pressure until the cellulose fibers of the wood have been freed or liberated from the encrusting or cementitious material by which they are bound together. 45 Thus, for example, I may employ a cooking liquor containing about 1.5% to 4.0% sodium sulphide, and about 2% to 5% sodium sulphite. In such case, the digestion 50 may be carried on in a closed digester from three to six hours, more or less, and at a

temperature as high as from 335° to 345° F., to yield a pulp having approximately the characteristics of kraft pulp, so-called.

The spent black liquor, which is separated from the pulp after the digesting operation and which contains the unspent sodium compounds, together with combustible organic compounds, and spent sodium in the form of various organic sodium compounds, is now treated in a manner to recover such compounds economically in a form for reutilization in the preparation of fresh cooking liquor. In such treatment, the waste liquor is evaporated to the desired degree of concentration, and is then delivered to a furnace 55 wherein its combustible organic content is burned and its inorganic or mineral content is smelted in a reducing atmosphere and recovered in a form suitable for the preparation of a fresh cooking liquor, that is, substantially in the form of sodium sulphide and sodium carbonate. The smelt taken from the furnace is dissolved in water and is then carbonated, as by bubbling carbon dioxide 60 through the aqueous solution, to cause the liberation of hydrogen sulphide from the sodium sulphide and, accordingly, the conversion of substantially the entire smelt solution to a solution of sodium carbonate. The sodium carbonate solution is then acidified 65 with sulphur dioxide to cause the liberation of carbon and the production of a solution of sodium sulphite. The carbon dioxide liberated during the acidification of the carbonate liquor is recovered and employed in 70 the carbonation of other smelt liquor, and the hydrogen sulphide liberated during such carbonation of the smelt liquor is recovered and employed in the preparation of the fresh cooking liquor. The hydrogen sulphide liberated 75 during the carbonation of the smelt liquor is recovered in the form of a sodium salt. For example, the recovered hydrogen sulphide may be caused to react with a caustic soda solution designed to replace sodium losses experienced in the cycle, thereby converting the caustic soda into sodium sulphide, 80 which is then mixed with the sulphite liquor resulting from the acidification of the carbonate liquor. When there is insufficient hy- 85

hydrogen sulphide available from the carbonation of the smelt liquor to effect a conversion of all the make-up caustic soda into sulphide, the cooking liquor will consist essentially of 5 a mixture of sodium sulphide, sodium sulphite, and caustic soda. If desired, the hydrogen sulphide liberated during the carbonation of the smelt solution may be burned to sulphur dioxide, which may be commingled 10 with other sulphur dioxide used to convert the carbonate solution into a sulphite solution; and the make-up caustic soda may be added, as such, to the sulphite solution to produce a digesting liquor containing essentially 15 only sodium sulphite and caustic soda as the pulping chemicals. Thus, the loss of sodium constituent in the cycle is compensated for by the addition of the necessary caustic soda, as previously indicated, and the loss 20 in sulphur constituent is made up during the acidification of the carbonate solution by the addition of sulphur dioxide produced by the combustion of sulphur or sulphur-bearing material. In fact, after the process is in 25 operation, practically the only chemicals which are needed for making up losses are sulphur or sulphur-bearing material and caustic soda.

The invention may best be understood from 30 the following more detailed disclosure thereof, when considered in conjunction with the accompanying drawing, which may be termed a "flow sheet" and in which I have illustrated diagrammatically and conventionally some 35 of the instrumentalities employed in the process and have indicated the course of the various solid, liquid and gaseous materials.

Referring to the drawing, at 1, I have 40 shown a digester which is preferably of the type usually employed for alkaline cooking. The digester is first filled with wood chips and the necessary quantity of alkaline liquor, e. g., a cooking liquor containing, say, 1.5% to 4% sodium sulphide and 2% to 5% sodium sulphite, is then pumped into the digester. The digester is then closed and its contents 45 are gradually heated to, say, 335° to 345° F., whereupon the cooking is continued for a period of time to ensure complete fiber liberation, tests being made in the usual manner from time to time until the cooking or fiber 50 liberation is judged to be complete.

After the cooking operation has been completed, the contents of the digester are blown 55 through a blow pipe 3, valved as at 4, into the usual blow pit indicated at 2. It is now necessary to separate the pulp from the spent liquor and to wash the pulp substantially free of such liquor and entrained products 60 of reaction prior to its passage through the usual screens which are employed for removing the so-called screenings therefrom, which consist of knots, shives, particles of brick, cement, etc. For this purpose, the pulp and 65 spent liquor associated therewith are re-

moved from the blow pit by a pump 5 through a pipe 5a and delivered to a washing machine consisting of a series of pulp washers indicated conventionally at 6. The washing machine is preferably of the counter-current type, substantially like that illustrated and described in U. S. Letters Patent No. 1,421,664, to Brown, Martinson, Moore & Parker, dated July 4, 1922, although, if desired, the ordinary rotary vacuum type of washer may be employed. In the washer of the patent referred to, the pulp is carried continuously through tanks in one direction, and the wash water is carried successively through such tanks in the opposite direction. The wash water is introduced through a pipe 7 to the pulp delivered at the last washer of the series, from which the washed pulp is delivered by a pump 8 through a conduit 9 to the usual screens (not shown). The wash water containing substantially all the spent liquor originally associated with the pulp is discharged from the first pulp washer of the series through a valved conduit 11 into a storage tank 13 which may also serve to receive spent liquor from the pipe 2a communicating with the bottom of the blow pit. It may be desirable to re-employ a portion of the spent black liquor, together with freshly prepared liquor, for the digestion of other raw cellulosic material, in which case spent liquor may be withdrawn through an outlet pipe 12 by a pump 14 and circulated to the digesters through a pipe 126.

At 15, I have illustrated conventionally a series of multiple effect evaporators, the details of construction of which it is unnecessary to describe, into the first effect 15a of which the spent liquor is delivered at the desired rate, by a pump 140, from the tank 13 through a pipe 16. While I preferably employ multiple effect evaporators, any other type of evaporator for removing a part of the aqueous content of the liquor may be used. From the last effect 15d of the evaporators, the liquor which has been concentrated to, say, about 16° Baumé, and which contains about 25% solids, is passed through a pipe 17 into a storage tank 18, from which it is withdrawn for the combustion of its organic content and the smelting of its inorganic compounds to form the sulphide and carbonate.

To this end, the concentrated spent liquor in the tank 18 is now subjected both to heat and pressure to generate an explosive effect therein, substantially as described in U. S. Letters Patent No. 1,326,414 to Moore and Quinn, dated December 30, 1919, and, as shown, is withdrawn from the tank 18 through a conduit 20 provided with a valve, as at 21, by a pump 22 a circulatory heating system including the pipe 23 and a heater 24. The liquor in passing through the sys-

tem is heated to a temperature above the boiling point by the heater 24, from which it passes through a pipe or series of valved pipes 25, terminating as nozzles 25a extending into a furnace, indicated as a whole at 26. In the present instance, it is desired that the sodium compounds recovered from the furnace should contain sodium sulphide and sodium carbonate. If this recovery takes place in a reducing atmosphere, there is no difficulty in recovering the desired salts, although, with these salts, there may be a slight amount of sodium sulphate, sodium sulphite, and caustic soda. In other words, the composition of the smelt is more or less comparable to that of the usual kraft or sulphate smelt.

The gas leaving the furnace contains some sulphur dioxide resulting from the decomposition of the sulphur compounds and also some sublimed sodium carbonate and sodium sulphide so that provision is made for the recovery of these chemicals. As shown, the gases emanating from the furnace are conducted through a stack 28 into the loose end of a scrubbing tower, indicated as a whole at 30, filled with inert interstitial material, and in counter-current flow to spent liquor diverted from the pipe 16 by a pipe 33 entering the upper end of the tower. The spent liquor dissolves the sulphur dioxide and the sublimed sodium salts of the furnace gases during its downward passage through the tower, and collects at the bottom of the tower, from which it is withdrawn and returned by a pipe 35 to the tank 13. Any gases which do not dissolve in the spent liquor circulated through the tower are permitted to emerge through a vent 30a.

The smelt produced in the furnace, consisting essentially of sodium sulphide and sodium carbonate, is delivered from spouts 36 to a dissolving tank 37 containing water supplied thereto at seasonable temperatures from a water conduit 39 provided with a valve indicated at 40. The smelt delivered from the furnace into the dissolving tank yields a hot solution which may contain a certain amount of solid impurities. Such impurities are preferably removed from the smelt liquor by filtration before the liquor is carbonated.

The carbonation of the smelt liquor may be accomplished either by bubbling carbon dioxide through the liquor or by causing such liquor and carbon dioxide to pass in counter-current flow through a suitable tower or series of towers packed with inert interstitial material. The smelt liquor contains, as already indicated, sodium carbonate and sodium sulphide, wherefore, the carbon dioxide by reaction with the sodium sulphide forms sodium carbonate and generates hydrogen sulphide.

In the present instance, the smelt liquor is withdrawn at the desired rate from the tank

87 for carbonation through a pipe 41 by a pump 42, which forces the liquor through a filter 43 and thence through a pipe 44 to the top of a carbonating tower, indicated as a whole at 45, which is packed with inert interstitial material.

In accordance with the present invention, I carbonate the smelt liquor with clean and substantially pure carbon dioxide obtained during the acidification of the sodium carbonate solution.

The carbon dioxide is passed into the lower end of the tower 45, and comes into intimate contact with the downwardly flowing smelt liquor. The rates of delivery of the smelt liquor and the carbon dioxide into the tower are controlled so that a liquor which is substantially entirely carbonated is produced without the introduction of excess carbon dioxide, wherefore the hydrogen sulphide liberated is not materially diluted by carbon dioxide.

The substantially pure hydrogen sulphide is conducted from the top of the tower 45 through a valved outlet pipe 47, into a gasometer indicated conventionally at 48, from which it is drawn for use either in converting to sodium sulphide the caustic soda liquor employed for making up losses in the cycle, or to be burned in air to sulphur dioxide, which is employed in the acidification of the carbonate liquor.

The carbonate liquor produced in the tower 45 collects at the bottom thereof, and is withdrawn through an outlet pipe 50 for delivery into a mixing tank 51 for conversion into sulphite. Before conducting the carbonate liquor into the mixing tank, however, it may be desirable to introduce a small quantity of chlorine into the pipe 50, as through a pipe 50a, to oxidize any residual sodium sulphide into sodium sulphite or sodium sulphate. This avoids reaction of the sodium sulphide with sulphur dioxide during acidification and the attendant formation of sodium thiosulphate or the precipitation of sulphur, either of which might give rise to objectionable mercaptan odors or the discoloration of the pulp during the digesting process.

In the practice of the present invention, I preferably employ the equivalent of a substantially pure sulphur dioxide for the acidification of the carbonate liquor. This may be had by treating such liquor with a solution of sulphurous acid produced, for example, by dissolving in water the products of combustion of the hydrogen sulphide liberated in the carbonating tower. Since practically no inert or insoluble gas accompanies a sulphurous acid solution, the carbon dioxide liberated from the carbonate liquor during acidification is practically undiluted by inert gas, and can consequently serve as the gas to be employed in the carbonating tower for the liberation of substantially pure hydrogen sulphide.

The sulphurous acid solution is delivered through a valved conduit 52 into the mixing tank 51 in amount sufficient to effect a complete conversion of the sodium carbonate to sodium sulphite without, however, introducing an excess which would dilute the carbon dioxide liberated thereby and rising to the top of the tank, from which it is delivered through the conduit 100 into the lower end of the carbonating tower. It is thus seen that the carbon dioxide liberated during the acidification of the sodium carbonate liquor is employed for the carbonation of the smelt liquor, and is again liberated as carbon dioxide during the acidification of the resulting carbonate solution.

The sulphurous acid solution employed for acidifying the carbonate solution can be prepared by dissolving in water sulphur dioxide obtained from any suitable source, as through the combustion of the recovered hydrogen sulphide or sulphur-bearing material. Any suitable method of forming a sulphurous acid solution may be employed, as by bubbling the sulphur dioxide through water (refrigerated, if desired, so as to secure a maximum concentration of  $\text{SO}_2$ ), or by passing it into counter-current contact with such water through one or more towers arranged in series. As shown on the drawing, sulphur is fed in molten state from the tank 55 into a rotary sulphur burner 56, wherein the sulphur is burned in the presence of atmospheric air, and wherefrom the products of combustion of the sulphur are conducted into a combustion chamber or stack 58, wherein the conversion of all sulphur vapor to sulphur dioxide is completed to form a gas comprising about 16% sulphur dioxide. The gas passes into a cooling and scrubbing tower indicated conventionally as a whole at 59, wherein the gases are more or less cooled and purified. The cooled gas is taken through a conduit 61 by a blower 62 and forced through a conduit 63 into the lower end of a tower indicated as a whole at 64, which is filled with a mass of inert interstitial material. The tower is supplied at its upper end with water from a valved pipe 65, the water absorbing the  $\text{SO}_2$  gas passed in counter flow thereto.

In case the hydrogen sulphide is burned and recovered as sulphur dioxide, the hydrogen sulphide stored in the gasometer 48 is taken therefrom at the desired pressure and velocity through a gas pipe or pipes 67, provided with regulating valves as at 67a, and terminating with nozzles or jets 68, which extend into a gas furnace indicated as a whole at 70. The hydrogen sulphide gas issuing from the nozzles is burned in the presence of air to form sulphur dioxide and water, the amount of air introduced into the furnace being accurately regulated to ensure complete combustion without the presence of unnecessary diluting air. The products

of combustion, after cooling, contain about 10% to 11%  $\text{SO}_2$  and may be commingled and employed together with the cooled and more or less purified sulphur burner gases in the preparation of a sulphurous acid solution. To this end, the combustion products of the hydrogen sulphide in the gas furnace 70 may pass therefrom through a conduit 71, and thence through a suitable cooler, for example, the double-pipe type worm cooler, indicated conventionally at 72. The water vapor contained in the products of combustion of the hydrogen sulphide is thus condensed from the  $\text{SO}_2$  gas, which is drawn by the blower 62 through the conduit 73 into the conduit 61 and mixed with the sulphur burner gas. By properly regulating the flow of gas from the sulphur dioxide sources and the rate of flow of water delivered into the tower 64, a 2% sulphurous acid solution is obtainable at the bottom of the tower. This solution can be taken from the tower through an outlet pipe 75 into a storage tank 76, from which it is drawn by a pump 77 and delivered through the pipe 52 into the mixing tank 51 in regulated amount. Any gases not absorbed by the sulphurous acid solution in the tower 64 are allowed to escape through a vent 176 at the top of the tower.

When all the hydrogen sulphide available from carbonation of the smelt liquor is burned to sulphur dioxide, the finished cooking liquor will be made up from the sodium sulphite solution in the mixing tank 51 and the caustic soda used for making up sodium losses occurring in the cycle. The sodium sulphite solution will in such case be conducted from the mixing tank through a valved pipe 177 to the storage tank 78, and the cooking liquor be finished by adding thereto sodium constituent in the form of caustic soda solution taken from a storage tank 80 through the valved pipe 81. The finished cooking liquor may then be withdrawn from the tank 78 by a pump 90 and conducted through a pipe 91 into the digester.

In certain cases, however, it may be desirable to provide a cooking liquor containing sodium sulphite and sodium sulphide or one containing sodium sulphite, sodium sulphide, and caustic soda. In such case, in place of burning the hydrogen sulphide to sulphur dioxide, the hydrogen sulphide is used in converting the caustic soda solution employed for making up losses in the cycle into sodium sulphide, as by bubbling the hydrogen sulphide thereinto, or by passing the caustic soda solution through one or more towers arranged in series in countercurrent contact with the hydrogen sulphide. As shown, the caustic soda solution is fed from a storage tank 83 into the upper end of an absorption tower, indicated generally at 85, and containing a mass of inert interstitial material. The lower end of the tower may be supplied with

hydrogen sulphide from a conduit 87 communicating with the conduit 47. The caustic soda liquor in passing downwardly through the tower undergoes neutralization by the hydrogen sulphide, resulting in a solution of sodium sulphide, which collects at the bottom of the tower and which may be conducted therefrom through a valved outlet pipe 88 to the tank 78, from which it may be withdrawn for use in the digesters. It is evident that if there is insufficient hydrogen sulphide available from the carbonating tower to convert all the caustic soda to sodium sulphide, the liquor leaving the tower 85 will consist of a mixture of sodium sulphide and caustic soda, so that the finished or prepared cooking liquor in the tank 78 for digesting the wood chips will consist essentially of sodium sulphite, sodium sulphide, and some caustic soda. Any inert gases accumulating at the top of the tower 85 may leave through the vent 85a.

By the control of the various instrumentalities employed in the process, one may adjust the quantities and relative proportions of sodium sulphite, sodium sulphide, and caustic soda in the finished cooking liquor. The higher the percentage of sodium sulphite or caustic soda, the closer the final pulp approaches kraft pulp in character. Inasmuch as there is a certain limiting amount of caustic soda which may be used to replace losses in the cycle, if the proportion of caustic soda in the cooking liquor is to be increased beyond this amount, it should be accomplished by the causticization of a portion of the carbonate liquor with lime. The preferred procedure, however, is one wherein all the caustic soda is converted into sodium sulphide by hydrogen sulphide, the remaining sodium in the cooking liquor being present in the form of sodium sulphite. Such a liquor has a less drastic effect on cellulosic material than when a portion of the make-up sodium constituent remains therein as caustic soda, and thus yields a stronger pulp which more closely approaches kraft pulps.

It is evident that in the practice of the process herein described, it is possible, though not ordinarily desirable, to recover a part of the hydrogen sulphide coming from the carbonating tower in the form of sulphur dioxide, and the remainder in the form of sodium sulphide, so that one may simultaneously practise both forms of sulphur recovery. The sulphur of the hydrogen sulphide is in any event recovered as a sodium-sulphur salt, to wit, either sodium sulphite or sodium sulphide, and thus is re-employed in the digesting operation. The cooking liquor is thus formed of a soluble sodium sulphur salt, e. g., sodium sulphite, and rendered alkaline by caustic soda, or sodium sulphide, or both, as hereinbefore pointed out. A slight amount of so-

dium sulphate may also be present, depending upon conditions of recovery.

What I claim is:

1. A process which comprises cooking raw cellulosic material in an alkaline solution of sodium sulphite; separating the pulp from the spent cooking liquor; smelting the inorganic content and burning the combustible content of such spent liquor; recovering the inorganicsmelted compounds; and passing the products of combustion from such smelting operation in contact with like spent liquor for the recovery of the soluble content of such products of combustion. 70

2. A process which comprises cooking raw cellulosic material in an alkaline solution of sodium sulphite; separating the pulp from the spent cooking liquor; burning the combustible content and smelting the inorganic content of such spent liquor in a reducing atmosphere in a manner to produce sodium sulphide and sodium carbonate; carbonating a solution of the smelt; and recovering the sulphur of the hydrogen sulphide liberated in such carbonation in the form of sodium sulphide. 80 85

3. A process which comprises concentrating and burning the combustible content and smelting the inorganic content of spent liquor resulting from the digestion of raw cellulosic material in an alkaline solution of sodium sulphite in a manner to produce sodium sulphide and sodium carbonate; recovering the smelted inorganic compounds in water; carbonating the smelt solution; recovering the sulphur of the hydrogen sulphide liberated in such carbonation in the form of a sodium salt; acidifying the carbonate solution with a solution of sulphurous acid; and recovering and utilizing the carbon dioxide liberated in such acidification in the carbonation of other smelt liquor. 95 100 105

4. A process which comprises concentrating and burning the combustible content and smelting the inorganic content of spent liquor resulting from the digestion of raw cellulosic material in an alkaline solution of sodium sulphite in a manner to produce sodium sulphide and sodium carbonate; recovering the smelted inorganic compounds in water; carbonating the smelt solution; recovering the sulphur of the hydrogen sulphide liberated in such carbonation in the form of sodium sulphide and sodium sulphite; acidifying the carbonate solution with sulphur dioxide; and recovering and utilizing the carbon dioxide liberated in such acidification in the carbonation of other smelt liquor. 110 115 120

5. A process which comprises concentrating and burning the combustible content and smelting the inorganic content of spent liquor resulting from the digestion of raw cellulosic material in an alkaline solution of sodium sulphite in a manner to produce sodium sulphide and sodium carbonate; recovering the 125

- smelting inorganic compounds in water; carbonating the smelt solution with substantially pure carbon dioxide and controlling such carbonation to produce substantially pure hydrogen sulphide; recovering the sulphur of the hydrogen sulphide liberated in such carbonation in the form of a sodium salt; acidifying the carbonate solution with a sulphurous acid solution formed from the products of combustion of sulphur-bearing material and controlling such acidification to produce a substantially pure carbon dioxide; and recovering and utilizing such carbon dioxide in the carbonation of other smelt liquor.
15. 6. A process which comprises concentrating and burning the combustible content and smelting the inorganic content of spent liquor resulting from the digestion of raw cellulosic material in an alkaline liquor containing sodium sulphite in a manner to produce sodium sulphide and sodium carbonate; recovering the smelted inorganic compounds in water; carbonating the smelt solution with substantially pure carbon dioxide and controlling such carbonation to produce substantially pure hydrogen sulphide; recovering such hydrogen sulphide; acidifying the carbonated solution with substantially pure sulphur dioxide to convert the sodium carbonate to sodium sulphite and controlling such acidification to produce a substantially pure carbon dioxide; utilizing such carbon dioxide in the carbonation of other smelt solution; treating a solution of caustic soda employed for making up losses in the process with said recovered hydrogen sulphide for conversion into sodium sulphide; mixing said treated solution with said sodium sulphite solution; and employing the mixed solution for the digestion of other raw cellulosic material.
7. A process which comprises digesting raw cellulosic material in an alkaline liquor containing sodium sulphite; concentrating and burning the combustible content and smelting the inorganic content of spent liquor resulting from such digestion in a manner to produce sodium sulphide and sodium carbonate; recovering the inorganic smelted compounds in water; carbonating the smelt solution with carbon dioxide and controlling such carbonation to produce substantially pure hydrogen sulphide and to effect a conversion of substantially all the sodium sulphide to sodium carbonate; recovering the sulphur of such hydrogen sulphide in the form of a sodium salt; acidifying the sodium carbonate solution with a solution of sulphur dioxide and controlling such acidification to produce a substantially pure carbon dioxide and a sodium sulphite solution; and utilizing the carbon dioxide obtained in such acidification for the carbonation of other smelt solution.
8. A process which comprises digesting raw cellulosic material in an alkaline cook-
- ing liquor containing sodium sulphite in solution; separating the pulp from the spent cooking liquor; smelting the inorganic content and burning the combustible content of such spent liquor in a manner to produce sodium sulphide and sodium carbonate; recovering the smelted inorganic compounds in water; carbonating the smelt solution with carbon dioxide; acidifying the carbonate solution with sulphur dioxide to produce a solution of sodium sulphide; recovering the hydrogen sulphite liberated in such acidification in the form of a sodium salt; and adding sodium constituent to said liquor in the form of caustic soda for making up losses in the cycle.
9. A process which comprises cooking raw cellulosic material in an alkaline solution of sodium sulphite and sodium sulphide; separating the pulp from the spent cooking liquor; smelting the inorganic content and burning the combustible content of such spent liquor in a reducing atmosphere to produce sodium sulphide; and recovering the inorganic smelted compounds for reuse in the cooking of other cellulosic material.
10. A process which comprises cooking raw cellulosic material in an alkaline cooking liquor containing sodium-sulphur compounds; separating the pulp from the spent cooking liquor; burning the combustible content and smelting the inorganic content of such spent liquor in a reducing atmosphere to form sodium sulphide; recovering the sodium sulphide in water; carbonating the sodium sulphide solution to sodium carbonate; and acidifying the carbonate solution with sulphur dioxide.
- In testimony whereof I have affixed my signature.
- GEORGE A. RICHTER.